

# UNITED STATES PATENT OFFICE.

GEORGE W. HOUSTON, OF MARIETTA, FLORIDA, ASSIGNOR TO HIMSELF,  
FRANK C. RAVESIES, OF OWENSBOROUGH, AND WILLIAM N. FERGUSON,  
OF DADE CITY, FLORIDA.

## PROCESS OF TANNING.

SPECIFICATION forming part of Letters Patent No. 623,403, dated April 18, 1899.

Application filed July 9, 1898. Serial No. 685,565. (No specimens.)

*To all whom it may concern:*

Be it known that I, GEORGE W. HOUSTON, of Marietta, in the county of Duval and State of Florida, have invented a new and Improved 5 Process of Tanning, of which the following is a full, clear, and exact description.

The object of my invention is to employ as a substitute for red-oak bark or any other 10 tanning agents usually employed an ooze made from a shrub commonly known as "horse-wickey" or "stagger-bush" and botanically designated as "*Pieris mariana*," which material will not only tan leather in 15 much less time than other material in common use, but is much more plentiful and economic and will produce a superior grade of leather at less expense.

A further object of the invention is to provide a tanning agent through the medium of 20 which the tanned leather may be given different shades of color, the shading being dependent upon the strength of the ooze and the character of the hide presented for tanning.

25 The invention consists in the novel steps of the process, to be hereinafter more fully set forth, and pointed out in the claims.

The hide to be tanned is trimmed to such an extent that it will be in good shape 30 and will be freed from all worthless encumbrances, and the hide is then placed in clear water, so as to thoroughly soften it. A solution is then made, composed, usually, of eight quarts of water and two quarts of lime, or 35 enough water to entirely cover the hides, the water and lime being in about the proportions above mentioned. The hides are then placed in this solution of lime until the hair slips. Usually about four days are necessary to ob-

tain this result with favorable weather. In 40 exceedingly cold weather a longer time is required. The hair is removed from the hides after the hides have been taken from the solution of lime, and said hair may be removed 45 by any suitable means—as, for instance, a currying-knife. The hides are then placed in clear water, and this bath is provided in order to soak out the greater portion of the lime from the hides. After the hides have

been taken from this water-bath they are 50 passed through powerful rollers or subjected to equivalent pressure for the purpose of partially drying the hides and removing entirely from them all the lime that they may still have retained. The hides are now in 55 condition to be subjected to the improved tanning agent, which is an ooze made from an herb known, respectively, as "horse-wickey," "stagger-bush," and "*Pieris mariana*." The ooze is made by boiling the shrub, 60 including the bark, wood, and leaves, or otherwise treating the said shrub to extract the strength therefrom in a liquid form. The ooze is made, preferably, very strong. In fact, it is preferably a saturated solution of 65 the shrub. In treating the hides with the improved tanning agent the hides are first placed in vats and are then soused in the ooze until the hides are covered about four inches. When the ooze is very powerful, the 70 hides should be frequently noticed, and then graded or classed after tanning. When the ooze is strong, ten days will be sufficient for the hides to remain in the ooze. According to the strength of the ooze and the character 75 or nature of the hides the tanned leather will be shaded light or dark, and such shading of the leather can only be accomplished successfully by practice in this particular method of tanning. The shades of the leather, however, 80 may be readily determined by closely watching the hides while in the ooze-bath. If a light-colored leather is desired, the hides are taken out as soon as the desired shade is obtained, and the longer the hides remain in 85 the ooze-bath the deeper and darker will be the shade obtained.

The amount of *Pieris mariana* used may be about one-half pound for every gallon of water; but it will be understood that the proportions may be varied considerably. Further, it will be obvious that the action of the tanning liquor produced from *Pieris mariana* according to my invention will remain substantially the same even when other substances are added to the tanning liquor as long as such substances do not affect the liquor detrimentally. The appended claims 95

are therefore to be interpreted as covering the extract of *Pieris mariana*, used either alone or with such other ingredients only that the tanning properties and advantages 5 of such extract will be availed of.

Having thus described my invention, I claim as new and desire to secure by Letters Patent—

1. The herein-described method of tanning leather, which consists in subjecting the hides, after preliminary treatment, to a bath containing an ooze made from an herb known as "horse-wickey," "stagger-bush" and "*Pieris mariana*," substantially as described.
- 15 2. A tanning liquor containing an ooze extracted from an herb known as "horse-

wickey," "stagger-bush" and "*Pieris mariana*," substantially as described.

3. A process of tanning leather, which consists in subjecting hides to a lime-bath, currying the hides, washing and compressing said hides to remove traces of lime, and finally subjecting the hides to a bath containing ooze obtained from a shrub known respectively as "horse-wickey," "stagger-bush" and "*Pie- 25*  
*ris mariana*," as set forth.

his  
GEORGE X W. HOUSTON.  
mark

Witnesses:

GEORGE WALSER,  
N. Y. BRYAN.